# EUROPEAN PATENT SPECIFICATION

(11) **EP 4 321 667 B1**
(45) Date of publication and mention of the grant of the patent: **18.02.2026**
(21) Application number: 23191163.7
(22) Date of filing: 11.08.2023
(51) Int. Cl.: D04H 1/56, D01D 5/08, D01F 1/10, D01F 6/14, D04H 3/007, D04H 3/16, D01D 5/098

(54) **POLYVINYL ALCOHOL FIBRES AND MELTBLOWN FIBROUS PRODUCTS**
POLYVINYLALKOHOLFASERN UND SCHMELZGEBLASENE FASERPRODUKTE
FIBRES D'ALCOOL POLYVINYLIQUE ET PRODUITS FIBREUX OBTENUS PAR FUSION-SOUFFLAGE

(30) Priority: 13.08.2022 EP 22190328
(43) Date of publication of application: 14.02.2024
(73) Proprietor: Aquapak IP Limited, Rubery Birmingham B31 5HE (GB)
(72) Inventor: WILLIAMS, John, Chirbury, SY15 6UD (GB); GRIFFITHS, Sian, Conwy, LL28 5LU (GB); ASHWORTH, Robert, Conwy, LL28 5YX (GB); EATON, Jack, Leeds, LS8 2AX (GB)
(74) Representative: Hepworth Browne

(56) References cited:
- JP-A- 2000 314 067
- JP-A- 2001 123 369
- US-A- 5 445 785
- US-A1- 2003 216 098
- US-A1- 2017 369 693

## Description

The invention relates to methods of manufacture of a nonwoven product comprising polyvinyl alcohol fibres and products incorporating such fibres.

Polyvinyl alcohol has many advantages in comparison to polymers which are traditionally used for manufacture of non-woven fibre products. Polyvinyl alcohol is soluble in water, particularly when heated, facilitating reclamation, recycling and environmental degradation.

Polyvinyl alcohol is manufactured by hydrolysis of homopolymer or co-polymers of polyvinyl acetate. Polyvinyl alcohol manufactured by partial or complete hydrolysis of homopolymeric polyvinyl acetate is referred to as homopolymeric polyvinyl alcohol. The degree of hydrolysis determines the properties of the resultant polymer. Co-polymeric polyvinyl alcohols or homopolymeric polyvinyl alcohol with a low degree (LD) of hydrolysis are easy to process but have inferior mechanical and chemical properties. Homopolymeric polyvinyl alcohol with a high degree (HD) of hydrolysis, for example 85% or greater, has superior properties but is not processable without degradation under conditions using apparatus employed for manufacture of polyolefin non-woven fibres.

Polyvinyl alcohol is soluble in water and fibres have traditionally been made by solution spinning methods using polyvinyl alcohol with a low degree (LD) of hydrolysis.

In order to enhance water resistance, thermal e.g. hot drawing and chemical e.g. acetylation steps have been required.

WO2017/046361 discloses a method for manufacture of processable polyvinyl alcohol having a degree of hydrolysis of 98% or greater.

WO2022/008521 discloses a method for manufacture of processable polyvinyl alcohol having a degree of hydrolysis in the range of 93% to 98% or more.

WO2022/008516 discloses a method for manufacture of plasticised polyvinyl alcohol having a degree of hydrolysis of 93% to 98% or more.

US5445785 discloses preparation of a non-woven web by extrusion of a solution of polyvinyl alcohol.

According to a first aspect of the present invention, there is provided a method of manufacture of a nonwoven product comprising polyvinyl alcohol fibres, the method comprising the steps of:
providing a polyvinyl alcohol composition comprising homopolymeric polyvinyl alcohol having a degree of hydrolysis of 88% to 98% or greater; and a weight average molecular weight in the range from 14,000 to 35,000;
wherein homopolymeric polyvinyl alcohol is made by hydrolysis of homopolymeric polyvinyl acetate;
a plasticiser selected from the group consisting of: diglycerol, triglycerol, fructose, ribose, xylose, D-mannitol, triacetin, pentaerythritol, dipentaerythritol, methyl pentanediol, 1,2-propanediol, 1,4-butanediol, 3-methyl-1,3-butanediol, 3,3-dimethyl-1,2-butanediol, polyethylene glycol 300, polyethylene glycol 400, alkoxylated polyethylene glycol, caprolactam, tricyclic trimethylolpropane formal, rosin esters, erucamide, and mixtures thereof; and
an optional stabilizer selected from the group consisting of: sodium stearate, potassium oleate, sodium benzoate, calcium stearate, stearic acid, dimethyl pentane diol, dimethyl propionic acid and mixtures thereof;
melting the composition at a temperature from 190°C to 240°C to form a molten polymer;
wherein the molten polymer is meltblown by the steps of:
   extrusion of the molten polymer through a die having a spinneret to form molten fibres of the polymer;
   the fibres being blown from the die and attenuated by a flow of heated air to form attenuated molten fibres, the attenuated fibres being deposited on a moving collector and allowed to solidify to form a melt blown nonwoven fibre web.

Melt blowing is a one step process which transforms a melt-processable polymer, particularly polyvinyl alcohol compositions for use in the method of this invention into non-woven fabric. Pellets of the polymer may be melted and the melt forced by spin pumps through spinnerets. containing multiple small orifices. The extruded polymer strands are attenuated just after the die using streams of hot air. The attenuated filaments are subsequently laid down on a collector to form a melt blown web, thus forming a self-bonded melt blown web composed of fine filaments of the polyvinyl alcohol composition. Melt blown non-woven fabrics are characterised as having very fine filaments, typically in the range 1 to 5µm.

For meltblown applications, the degree of hydrolysis may be 90-95%, preferably 93-95%.

For meltblown applications, the molecular weight of the homopolymeric polyvinyl alcohol may be in the range from 14,000 to 22,000, for example, 15,000 to 20,000, for example 16,000 to 20,000.

Molecular weights in this specification are weight average molecular weights and are measured using conventional liquid chromatographic techniques.

In embodiments, the composition may be melted at a temperature from 220°C to 240°C.

The polyvinyl alcohol composition for use in the method of this invention may have a melt flow index (MFI) of 30 to 80g/10min, for example 50 to 75g/10min, for example 70 to 75g/10min. Melt flow indices referred to in this specification are determined at 230°C using a weight of 10kg by conventional techniques.

The polyvinyl alcohol composition for use in the method of this invention is stable at the temperature at which it is melted and extruded. Polyvinyl alcohol, not containing a plasticiser and stabiliser as disclosed herein, particularly the homopolymer having a high degree of hydrolysis, may be liable to decompose at the temperatures required for melting and extrusion processing.

Advantageous polyvinyl alcohol fibres for use in this invention are capable of being processed on a commercial scale, using conventional meltblowing apparatus.

The stabilised polyvinyl alcohol polymers used in this invention may be manufactured in accordance with WO2022/008516 and WO2022/008521.

The polyvinyl alcohol composition may be made by a method comprising the steps of:
introducing into a mixing reactor a polyvinyl alcohol polymer comprising homopolymeric polyvinyl alcohol or a blend thereof having a degree of hydrolysis in the range of 88 wt% to 98 wt% or more;
wherein the mixing reactor comprises a blending chamber having a primary inlet, a primary outlet and at least two inter-engaging components extending between the primary inlet and primary outlet, the components being arranged to apply a shearing force to the polymer while the polymer is conveyed by the components from the inlet through a reaction zone to the outlet;
one or more secondary inlets located downstream from the primary inlet for introducing reactants comprising a processing aid, a plasticiser and an optional reactive stabiliser to the chamber to form a reaction mixture;
wherein the plasticiser is selected from the group disclosed above;
wherein the reactive stabiliser when present is selected from the group consisting of:
   sodium stearate, potassium oleate, sodium benzoate, calcium stearate, stearic acid, dimethyl propionic acid, and mixtures thereof;
   wherein the blending chamber comprises a plurality of heated regions arranged so that the mixture is subjected to a temperature profile whereby the temperature increases from the inlet to the outlet;
   a secondary outlet located between the reaction zone and primary outlet arranged to allow removal of processing aid from the chamber;
   reacting the processing agent, plasticiser and polymer in the reaction zone to form plasticised polymer; and
   allowing the plasticised polymer to pass from the primary outlet.

Use of a reactive mixing apparatus, typically an extruder for use in accordance with this invention allows the processing aid and plasticiser to be reacted with the polyvinyl alcohol or blend thereof, without decomposition of the polymer followed by removal of all or most of the processing aid from the secondary outlet to give plasticised polyvinyl alcohol or a blend thereof.

Use of a reactive stabiliser may result in an advantageous reduction in the extent of degradation during melt processing. This allows homopolymeric polyvinyl alcohol having a high degree of hydrolysis, for example 88 wt% or higher to be processed to form fibres or pellets from which fibres may be formed by extrusion.

The reactive stabiliser may be used in an amount of about 0.1 wt% to about 5 wt%, for example about 0.1 wt% to about 3 wt%, for example 0.1 wt% to about 1.5 wt%, for example from about 0.2 wt% to about 0.5 wt%, for example about 0.25 wt%.

Homopolymeric polyvinyl alcohol has been difficult to process due to degradation at the high temperatures required. The liability of degradation has led to use of polyvinyl alcohol co-polymers with a consequent loss of engineering properties. This can be seen by UV spectral analysis of the amount of conjugation present in the polymer. Sodium benzoate has been found to be particularly effective.

Use of homopolymeric polyvinyl alcohol is particularly advantageous. Homopolymeric polyvinyl alcohol is manufactured by hydrolysis of homopolymeric polyvinyl acetate, the degree of hydrolysis being 90wt% or more in embodiments of this invention. Polyvinyl alcohol co-polymers made by hydrolysis of polyvinyl acetate co-polymers have inferior properties compared to homopolymeric polyvinyl alcohol. Homopolymeric polyvinyl alcohol may exhibit advantageous properties.

Polyvinyl alcohol polymers for use in this invention may have high tensile strength and flexibility.

The polyvinyl alcohol may be manufactured by hydrolysis of homopolymeric polyvinyl acetate, wherein the extent of hydrolysis is in the range from 88 wt% up to 98 wt%, for example 90 wt% to less than 95 wt%.

A blend of two or more polyvinyl alcohol polymers may be employed, for example a blend of two polyvinyl alcohol polymers with a relatively high molecular weight and a relatively low molecular weight respectively.

A blend of polyvinyl alcohols with the same molecular weight and different degrees of hydrolysis can be combined. Blending different polyvinyl alcohol grades together enables the properties of the resultant polymer to be enhanced, for example melt strength.

For fibre production a blend of two polyvinyl alcohol polymers with a molecular weight in the range 14,000 to 22,000, a first polymer having a low degree of hydrolysis and a second polymer having a high degree of hydrolysis may be blended in a ratio of 40:60 to 60:40, for example about 50:50 by weight.

The blends of different molecular weight polymers employed are selected in accordance with the physical properties required in the finished product. This may require different molecular weight materials being used. Use of more than two different molecular weight polymers may be advantageous. The use of a single molecular weight polymer is not precluded.

Use of a blend may allow control of the viscosity of the polymer. Selection of a stabiliser in accordance with the present invention allows use of blends of a desired viscosity without a loss of other properties. Alternatively, use of a blend may permit use of polyvinyl alcohol with one or more stabilisers while maintaining viscosity or other properties to permit manufacture of pellets or films.

The processing aid is preferably water. Alternatively, the processing aid may comprise a mixture of water and one or more hydroxyl compound with a boiling point less than the boiling point or melting point of the plasticiser. Use of water is preferred for cost and environmental reasons.

Two or more plasticisers may be employed.

When a mixture of plasticisers is employed, a binary mixture may be preferred.

In an embodiment, the plasticiser may be selected from the group consisting of: diglycerol, triglycerol, xylose, D-mannitol, triacetin, dipentaerythritol, 1,4-butanediol, 3,3-dimethyl-1,2-butanediol, and caprolactam.

The total amount of plasticiser in the formulation may be from about 15 wt% to about 30 wt%.

Polymer compositions and fibres for use in the present invention may not include any or any substantial amount of a water soluble salt, oil, wax or ethylene homopolymer or copolymer.

The method of this invention provides many advantages. The method allows formation of thermally processable polyvinyl alcohol which can be used to create economical fibres that are highly functional while eliminating plastic pollution. Polyvinyl alcohol is water-soluble, non-toxic to the environment and inherently biodegradable. Hydrophilic polymers, for example, polyvinyl alcohol degrade environmentally faster than hydrophobic polymers and do not show bioaccumulation. Thermoplastic polyvinyl alcohol can be mechanically recycled into pellets for repeated use.

Homopolymeric polyvinyl alcohol fibres for use in this invention provide many advantages in comparison to previously available polyvinyl alcohol containing fibres. The fibres of this invention and products made from these fibres exhibit improved tensile strength, barrier properties, water solubility and biodegradability. Homopolymeric polyvinyl alcohol fibres may unexpectedly exhibit all of these properties. In comparison, copolymers have only been able to compromise and provide one or more of these properties at the expense of other properties. The fibres and products of the present invention have a desirable monomaterial structure which does not suffer from this disadvantage.

The fibres for use in this invention may exhibit advantageous chemical resistance, particularly to alcohols, acids and alkalis.

Meltblown fibres for use in this invention may have an advantageous smaller diameter. Fibres having a smaller diameter have a greater surface area which may be advantageous for air filtration, for example in face masks. Finer fibres may also be softer in texture. Furthermore, finer fibres may also have an increased rate of biodegradation after use.

According to a second aspect of the present disclosure there is provided meltblown homopolymeric polyvinyl alcohol fibre having a degree of hydrolysis of 88 wt% to 98 wt% or greater. The fibre may be manufactured in accordance with the first aspect of the present invention.

According to a third aspect of the present invention, there is provided a meltblown non-woven fibre product comprising fibres of homopolymeric polyvinyl alcohol having a degree of hydrolysis of 88 wt% to 98 wt% or greater. The product is made in accordance with the method of the first aspect of the present invention.

A non-woven product is defined by ISO9092 as an engineered fibrous assembly, primarily planar, which has been given a designed level of structural integrity by physical and/or chemical means, excluding weaving, knitting or paper making.

The areal density may be about 50gm⁻², dependent on the application, for example single or multiple use applications.

In embodiments, the areal density may be about 60gm⁻². Non woven fabrics having this density may be employed for manufacture of flushable wipes.

The following processing parameters may be employed.

The die temperature may be in the range 200°C to 230°C. An optimal die temperature may be 220°C. Melt breaks may be observed at higher temperatures.

The air flow volume may be in the range 2,000 to 7,000 1 min⁻¹, for example 5,900 to 6,900 1 min⁻¹. A higher air flow of 7,000 1 min⁻¹ may allow greater drawing of the polymer stream and may allow the average filament diameter to be reduced from 14.1µm to 12.6µm.

The die air temperature may be in the range 200 to 280°C, for example 245 to 280°C. A preferred air temperature may be 220 to 240°C. An increase to a higher die air temperature may result in more frequent melt breaks. A die-to-collector distance of 0.1 to 0.25m, for example 0.24m may be employed.

Meltblown polyvinyl alcohol nonwoven fabrics of this invention find many applications which utilise the unique properties of homopolymeric polyvinyl alcohol.

Percentages and other quantities referred to in this specification are by weight unless stated otherwise and are selected from any ranges quoted to total 100%.

The invention is further described by means of example but not in any limitative sense, with reference to the accompanying drawings, of which:
Figure 1 is a diagrammatic view of meltblowing apparatus for use in accordance with this invention; and
Figure 2 is a cross sectional view of the die of the apparatus shown in Figure 1.

In embodiments of the present invention the following polyvinyl alcohol (PVOH) homopolymer compositions may be employed. Compositions A and B are not for use in the method of the invention.

### Polymer composition A

| | |
|---|---|
| PVOH; degree of hydrolysis 98%; low viscosity | 35.97% |
| PVOH; degree of hydrolysis 89%; low viscosity | 35.97% |
| Trimethylol propane | 14.37% |
| Sodium benzoate | 0.21% |
| Glycerol | 4.29% |
| Water | 9.20% |

### Polymer composition B

| | |
|---|---|
| PVOH; degree of hydrolysis 99%; high viscosity | 7.193% |
| PVOH; degree of hydrolysis 98%; low viscosity | 64.737% |
| Trimethylol propane | 14.37% |
| Sodium benzoate | 0.21 |
| Glycerol | 4.29% |
| Water | 9.20% |

### Polymer composition C

| | |
|---|---|
| PVOH; degree of hydrolysis 98%; low viscosity | 35.87% |
| PVOH; degree of hydrolysis 89%; low viscosity | 35.87% |
| Di-pentaerythritol | 6.21% |
| Triacetin | 12.41% |
| Sodium benzoate | 0.25% |
| Water | 9.39% |

### Polymer composition D

| | |
|---|---|
| PVOH; degree of hydrolysis 98%; low viscosity | 22.61% |
| PVOH; degree of hydrolysis 97%; medium viscosity | 52.76% |
| Dipentaerythritol | 4.99% |
| Sodium benzoate | 0.25% |
| Triacetin | 10.00% |
| Water | 9.39% |

### Polymer composition E

| | |
|---|---|
| PVOH; degree of hydrolysis 98%; low viscosity | 25.20% |
| PVOH; degree of hydrolysis 98%; low viscosity | 5.20% |
| PVOH; degree of hydrolysis 89%; low viscosity | 25.21% |
| Dipentaerythritol | 5.00% |
| Triacetin | 10.00% |
| Water | 9.39% |

### Polymer composition F

| | |
|---|---|
| PVOH; degree of hydrolysis 98%; low viscosity | 27.33% |
| PVOH; degree of hydrolysis 98%; low viscosity | 27.33% |
| PVOH; degree of hydrolysis 89%; low viscosity | 27.33% |
| Dipentaerythritol | 8.00% |
| Methyl pentanediol | 5.50% |
| Glycerol | 4.50% |

### Polymer composition G

| | |
|---|---|
| PVOH; degree of hydrolysis 98%; low viscosity | 72.45% |
| PVOH; degree of hydrolysis 99%; high viscosity | 9.20% |
| Dipentaerythritol | 7.95% |
| Methyl pentanediol | 5.63% |
| Glycerol | 4.50% |
| Sodium benzoate | 0.27% |

Figures 1 and 2 illustrate meltblowing apparatus used in accordance with the present invention.

An extruder (1) supplies molten polyvinyl alcohol composition to a gear pump (2) which feeds the polymer to a die (3). Air manifolds (4) supply primary high velocity air flows to the die outlet (5) so that the primary air flows surround the die outlet (6) of the polymer feed (7). The primary air flows create a stream of molten fibres (8) directed towards a rotating cylindrical collector (9). Secondary air flows (10) serve the cool the streams of molten polymer fibres, promoting solidification of the polymer streams as they contact the collector (9) to form a solidified non-woven web (11). The solidified web (11) is drawn from the collector and wound upon a rotary winder (12).

### Example 1 - not according to the invention.

Meltblown polyvinyl alcohol fibres were extruded using the following parameters.

Meltblowing of a polyvinyl alcohol composition was carried out using the following parameters. Polymer composition A was employed.

### Meltblowing parameters

| Parameters | |
|---|---|
| Extruding zone 1 | 180°C |
| Extruding zone 2 | 200°C |
| Extruding zone 3 | 205°C |
| Die temperature | 210-220°C |
| Air temperature | 240-280°C |
| Air flow volume | 6900 1.min⁻¹ |
| Die-to-collector distance | 0.1-0.3m |
| Extrusion speed | 6-16rpm |
| Die hole diameter | 0.25mm |
| Air angle | 45° |
| Air knife gap | 0.7-1.4mm |

An advantageous polyvinyl alcohol polymer for formation of melt blown fabrics had a degree of hydrolysis of 94%, using trimethylolpropane as a plasticiser with additional glycerol.

The resultant meltblown fabrics had an areal density of 60.88g/m², thickness of 0.51mm; filament diameter of 12.61µm; air impermeability at 200 Pa of 3,536 1.min⁻² s⁻¹ and tensile strength, MD of 0.44 l/25mm, before thermal bonding.

A significant proportion (65%) of the filament diameters was measured between 5 and 14µm with an average filament diameter of 12.6µm. The air velocity was 6,900 l.min⁻¹ at an air flow of 6,200 l.min⁻¹, a significant proportion of the filament diameters was between 10 and 14µm with an average filament diameter of 14.12µm. Higher air velocity allowed attenuation of the polymers into fine filaments.

## Claims

1. A method of manufacture of a nonwoven product comprising polyvinyl alcohol fibres, the method comprising the steps of:
providing a polyvinyl alcohol composition comprising homopolymeric polyvinyl alcohol having a degree of hydrolysis of 88% to 98% or greater; and a weight average molecular weight in the range from 14,000 to 35,000;
wherein the homopolymeric polyvinyl alcohol is made by hydrolysis of homopolymeric polyvinyl acetate;
a plasticiser selected from the group consisting of: diglycerol, triglycerol, fructose, ribose, xylose, D-mannitol, triacetin, pentaerythritol, dipentaerythritol, methyl pentanediol, 1,2-propanediol, 1,4-butanediol, 3-methyl-1,3-butanediol, 3,3-dimethyl-1,2-butanediol, polyethylene glycol 300, polyethylene glycol 400, alkoxylated polyethylene glycol, caprolactam, tricyclic trimethylolpropane formal, rosin esters, erucamide, and mixtures thereof; and
an optional stabilizer selected from the group consisting of: sodium stearate, potassium oleate, sodium benzoate, calcium stearate, stearic acid, dimethyl pentane diol, dimethyl propionic acid and mixtures thereof;
melting the composition at a temperature from 190°C to 240°C to form a molten polymer;
wherein the molten polymer is meltblown by the steps of:
extrusion of the molten polymer through a die having a spinneret to form molten fibres of the polymer;
the fibres being blown from the die and attenuated by a flow of heated air to form attenuated molten fibres, the attenuated fibres being deposited on a moving collector and allowed to solidify to form a melt blown nonwoven fibre web.

2. A method as claimed in claim 1, wherein the plasticiser is selected from the group consisting of: diglycerol, triglycerol, D-mannitol, triacetin, dipentaerythritol, caprolactam and mixtures thereof.

3. A method as claimed in claim 1, wherein the optional stabiliser is selected from the group consisting of: sodium stearate, potassium oleate, sodium benzoate, calcium stearate and mixtures thereof.

4. A method as claimed in any preceding claim, wherein the degree of hydrolysis is 90 to 95wt%.

5. A method as claimed in claim 4, wherein the degree of hydrolysis is 93 to 95wt%.

6. A method as claimed in any preceding claim, wherein the molecular weight of the homopolymeric polyvinyl alcohol is in the range of 14,000 to 22,000.

7. A method as claimed in claim 6, wherein the molecular weight of the homopolymeric polyvinyl alcohol is in the range of 15,000 to 20,000.

8. A method as claimed in claim 7, wherein the molecular weight of the homopolymeric polyvinyl alcohol is in the range of 16,000 to 20,000.

9. A method as claimed in any preceding claim, wherein the composition is melted at a temperature in the range from 220°C to 230°C.

10. A method as claimed in any preceding claim, wherein the polyvinyl alcohol composition has a melt flow index in the range of 30 to 80g/10min.

11. A method as claimed in claim 10, wherein the polyvinyl alcohol composition has a melt flow index in the range of 50 to 75g/10min.

12. A method as claimed in claim 11, wherein the polyvinyl alcohol composition has a melt flow index in the range of 70 to 75g/10min.

13. A method as claimed in any preceding claim, wherein the molten polymer is extruded from a die having a temperature in the range of 200°C to 220°C.

14. A method as claimed in any preceding claim, wherein the air temperature at the die is in the range of 200°C to 280°C.

15. A method as claimed in any preceding claim, wherein the air pressure at the die is 50 kPa to 110 kPa.

16. A method as claimed in any preceding claim, wherein the fibre diameter is in the range of 12 µm to 15 µm.

17. A meltblown nonwoven fabric comprising homopolymeric polyvinyl alcohol having a degree of hydrolysis of 88 wt% to 98 wt% or greater, made by the method of any of claims 1 to 16.

18. A product incorporating a meltblown fabric as claimed in claim 17, wherein the product is selected from the group consisting of: dry wipes, hygiene top sheets and core wraps, filters, face masks and personal protective equipment.

## Patentansprüche

1. Verfahren zur Herstellung eines Vliesprodukts mit Polyvinyl-Alkohol-Fasern,
wobei das Verfahren die Schritte enthält:
Vorsehen einer Polyvinyl-Alkoholzusammensetzung, wobei die Zusammensetzung homopolymeren Polyvinyl-Alkohol mit einem Hydrolysegrad von 88% bis 98% oder höher und ein durchschnittliches Molekulargewicht im Bereich von 14.000 bis 35.000 enthält;
wobei der homopolymere Polyvinyl-Alkohol durch Hydrolyse von homopolymerem Polyvinylazetat hergestellt ist;
eines Weichmachers ausgewählt aus einer Gruppe bestehend aus: Diglyzerin, Triglyzerin, Fructose, Ribose, Xylose, D-Mannit, Triacetin, Pentaerythrit, Dipentaerythrit, Methyl-Pentandiol, 1,2-Propandiol, 1,4-Butandiol, 3-Methyl-1,3-Butandiol, 3,3-Dimethyl-1,2-Butandiol, Polyethylenglykol 300, Polyethylenglykol 400, alkoxyliertes Polyethylenglykol, Caprolactam, trizyklisches Trimethylolpropanformal, Harzester, Erucasäureamid und Mischungen davon; und
einen optionalen Stabilisator ausgewählt aus der der Gruppe bestehend aus: Natriumstearat, Kaliumoleat, Natriumbenzoat, Calciumstearat, Stearinsäure, Dimethylbutandiol, Dimethylpropionsäure und Mischungen davon;
Schmelzen der Zusammensetzung bei einer Temperatur von 190°C bis 240°C zum Formen eines geschmolzenen Polymers;
wobei das geschmolzene Polymer in den folgenden Schritten schmelzgesponnen wird:
Extrusion des geschmolzenen Polymers durch eine Düse mit einer Spinndüse zum Formen geschmolzener Fasern aus dem Polymer;
wobei die Fasern aus der Düse geblasen werden und von einem Strom geheizter Luft verdünnt werden zum Formen von verdünnten, geschmolzenen Fasern, wobei die verdünnten Fasern auf einem bewegten Kollektor abgelegt werden und erstarren gelassen werden zum Formen eines schmelzgesponnenes Vliesfasergewebes.

2. Verfahren nach Anspruch 1, wobei der Weichmacher ausgewählt ist aus der Gruppe bestehend aus: Diglyzerin, Triglyzerin, D-Mannit, Triacetin, Dipentaerythrit, Caprolactam und Mischungen davon.

3. Verfahren nach Anspruch 1,
wobei der optionale Stabilisator ausgewählt ist aus der Gruppe bestehend aus:
Natriumstearat, Kaliumoleat, Natriumbenzoat, Calciumstearat und Mischungen davon.

4. Verfahren nach einem der vorhergehenden Ansprüche, wobei der Hydrolysegrad 90 bis 95 Gew.% beträgt.

5. Verfahren nach Anspruch 4, wobei der Hydrolysegrad 93 bis 95 Gew.% beträgt.

6. Verfahren nach einem der vorhergehenden Ansprüche, wobei das Molekulargewicht des homopolymeren Polyvinyl-Alkohol im Bereich von 14.000 bis 22.000 liegt.

7. Verfahren nach Anspruch 6, wobei das Molekulargewicht des homopolymeren Polyvinyl-Alkohol im Bereich von 15.000 bis 20.000 liegt.

8. Verfahren nach Anspruch 7, wobei das Molekulargewicht des homopolymeren Polyvinyl-Alkohol im Bereich von 16.000 bis 20.000 liegt.

9. Verfahren nach einem der vorhergehenden Ansprüche, wobei die Zusammensetzung bei einer Temperatur im Bereich von 220°C bis 230°C geschmolzen wird.

10. Verfahren nach einem der vorhergehenden Ansprüche, wobei die Polyvinyl-Alkoholzusammensetzung einen Schmelzflussindex im Bereich von 30 bis 80g/10min hat.

11. Verfahren nach Anspruch 10, wobei die Polyvinyl-Alkoholzusammensetzung einen Schmelzflussindex im Bereich von 50 bis 75g/10min hat.

12. Verfahren nach Anspruch 11, wobei die Polyvinyl-Alkoholzusammensetzung einen Schmelzflussindex im Bereich von 70 bis 75g/10min hat.

13. Verfahren nach einem der vorhergehenden Ansprüche, wobei das geschmolzene Polymer aus einer Düse extrudiert wird, die eine Temperatur im Bereich von 200°C bis 220°C hat.

14. Verfahren nach einem der vorhergehenden Ansprüche, wobei die Lufttemperatur an der Düse im Bereich von 200°C bis 280°C liegt.

15. Verfahren nach einem der vorhergehenden Ansprüche, wobei der Luftdruck an der Düse 50 kPa bis 110 kPa beträgt.

16. Verfahren nach einem der vorhergehenden Ansprüche, wobei der Faserdurchmesser im Bereich von 12 µm bis 15 µm liegt.

17. Schmelzgesponnenes Gelege, enthaltend homopolymeren Polyvinyl-Alkohol, der einen Hydrolysegrad von 88 Gew.% bis 98 Gew.% oder höher hat, hergestellt durch ein Verfahren nach einem der Ansprüche 1 bis 16.

18. Produkt, das ein schmelzgesponnenes Gelege nach Anspruch 17 beinhaltet, wobei das Produkt ausgewählt ist aus der Gruppe bestehend aus: Trockentücher, Hygieneoberschichten, Kernummantelungen, Filter, Gesichtsmasken und Personenschutzausrüstung.

## Revendications

1. Procédé de fabrication d'un produit non-tissé comprenant des fibres d'alcool polyvinylique, le procédé comprenant les étapes de :
mise à disposition d'une composition d'alcool polyvinylique comprenant de l'alcool polyvinylique homopolymère présentant un degré d'hydrolyse de 88 % à 98 % ou plus ; et une masse molaire moyenne en masse dans la plage de 14 000 à 35 000 ;
selon lequel l'alcool polyvinylique homopolymère est obtenu par hydrolyse d'acétate polyvinylique homopolymère ;
un plastifiant choisi dans le groupe consistant en : le diglycérol, le triglycérol, le fructose, le ribose, le xylose, le D-mannitol, la triacétine, le pentaérythritol, le dipentaérythritol, le méthylpentanediol, le 1,2-propanediol, le 1,4-butanediol, le 3-méthyl-1,3-butanediol, le 3,3-diméthyl-1,2-butanediol, le polyéthylène glycol 300, le polyéthylène glycol 400, le polyéthylène glycol alcoxylé, le caprolactame, le formal de triméthylolpropane tricyclique, les esters de colophane, l'érucamide, et des mélanges de ceux-ci ; et
un stabilisant optionnel choisi dans le groupe consistant en : le stéarate de sodium, l'oléate de potassium, le benzoate de sodium, le stéarate de calcium, l'acide stéarique, le diol de diméthylpentane, l'acide propionique diméthylique et des mélanges de ceux-ci ;
fusion de la composition à une température de 190 °C à 240 °C afin de former un polymère en fusion ;
selon lequel le polymère en fusion est soufflé-extrudé via les étapes de :
extrusion du polymère à travers une matrice présentant une filière afin de former des fibres de polymère en fusion ;
les fibres étant soufflées depuis la matrice et atténuées par un flux d'air chaud afin de former des fibres, en fusion, atténuées, les fibres atténuées étant déposées sur un collecteur mobile et solidifiées de manière à former une nappe de fibres non-tissées à extrusion soufflée.

2. Procédé selon la revendication 1, selon lequel le plastifiant est choisi dans le groupe consistant en : le diglycérol, le triglycérol, le D-mannitol, la triacétine, le dipentaérythritol, le caprolactame et des mélanges de ceux-ci.

3. Procédé selon la revendication 1, selon lequel le stabilisant optionnel est choisi dans le groupe consistant en : le stéarate de sodium, l'oléate de potassium, le benzoate de sodium, le stéarate de calcium, et des mélanges de ceux-ci.

4. Procédé selon l'une quelconque des revendications précédentes, selon lequel le degré d'hydrolyse est de 90 à 95 % en poids.

5. Procédé selon la revendication 4, selon lequel le degré d'hydrolyse est de 93 à 95 % en poids.

6. Procédé selon l'une quelconque des revendications précédentes, selon lequel la masse molaire de l'homopolymère d'alcool polyvinylique se situe dans la plage de 14 000 à 22 000.

7. Procédé selon la revendication 6, selon lequel la masse molaire de l'homopolymère d'alcool polyvinylique se situe dans la plage de 15 000 à 20 000.

8. Procédé selon la revendication 7, selon lequel la masse molaire de l'homopolymère d'alcool polyvinylique se situe dans la plage de 16 000 à 20 000.

9. Procédé selon l'une quelconque des revendications précédentes, selon lequel la composition est mise en fusion à une température se situant dans la plage de 220 °C à 230 °C.

10. Procédé selon l'une quelconque des revendications précédentes, selon lequel la composition d'alcool polyvinylique présente un indice de fluidité à chaud se situant dans la plage de 30 à 80 g / 10 min.

11. Procédé selon la revendication 10, selon lequel la composition d'alcool présente un indice de fluidité à chaud se situant dans la plage de 50 à 75 g / 10 min.

12. Procédé selon la revendication 11, selon lequel la composition d'alcool polyvinylique présente un indice de fluidité à chaud se situant dans la plage de 70 à 75 g / 10 min.

13. Procédé selon l'une quelconque des revendications précédentes, selon lequel le polymère en fusion est extrudé d'une matrice présentant une température dans la plage de 200 °C à 220 °C.

14. Procédé selon l'une quelconque des revendications précédentes, selon lequel la température de l'air au niveau de la matrice se situe dans la plage de 200 °C à 280 °C.

15. Procédé selon l'une quelconque des revendications précédentes, selon lequel la pression d'air au niveau de la matrice est de 50 kPa à 110 kPa.

16. Procédé selon l'une quelconque des revendications précédentes, selon lequel le diamètre de fibre se situe dans la plage de 12 pm à 15 pm.

17. Textile non-tissé soufflé-extrudé comprenant de l'alcool polyvinylique homopolymère présentant un degré d'hydrolyse de 88 % en poids ou plus, obtenu par le procédé selon l'une quelconque des revendications 1 à 16.

18. Produit incorporant un textile soufflé-extrudé selon la revendication 17, selon lequel le produit est choisi dans le groupe consistant en : lingettes sèches, draps de dessus et enveloppes d'âme hygiéniques, des filtres, des masques de protection faciale et de l'équipement de protection personnelle.
